



US006997234B2

(12) **United States Patent**  
Peterson

(10) Patent No.: **US 6,997,234 B2**  
(45) Date of Patent: **Feb. 14, 2006**

(54) **ENHANCED GRAVITY CASTING**

(75) Inventor: **Norman E. Peterson**, Wyoming, MN (US)

(73) Assignee: **Water Gremlin Company**, White Bear Lake, MN (US)

(\*) Notice: Subject to any disclaimer, the term of this patent is extended or adjusted under 35 U.S.C. 154(b) by 92 days.

(21) Appl. No.: **10/673,710**

(22) Filed: **Sep. 29, 2003**

(65) **Prior Publication Data**

US 2005/0067132 A1 Mar. 31, 2005

(51) **Int. Cl.**  
**B22D 27/15** (2006.01)

(52) **U.S. Cl.** **164/133; 164/120; 164/61**

(58) **Field of Classification Search** **164/113, 164/120, 61, 133, 136**

See application file for complete search history.

(56) **References Cited**

**U.S. PATENT DOCUMENTS**

4,377,197 A \* 3/1983 Oxenreider et al. .... 164/112  
5,244,033 A \* 9/1993 Ueno ..... 164/312  
6,564,853 B1 \* 5/2003 Ratte ..... 164/113

**FOREIGN PATENT DOCUMENTS**

CH 321596 5/1957  
FR 2504424 10/1982  
GB 1257963 12/1971

\* cited by examiner

*Primary Examiner*—Jonathan Johnson

*Assistant Examiner*—Len Tran

(74) *Attorney, Agent, or Firm*—Jacobson & Johnson

(57) **ABSTRACT**

An apparatus and method for enhanced gravity casting wherein a portion of the mold is maintained in pressure contact with molten metal as it solidifies to allow the mold surface to follow the contraction of the solidifying metal. A further feature of the invention is the use of an air clearance between mold parts that is sufficient to allow air to escape but insufficient to allow molten metal to flow therewith.

**9 Claims, 2 Drawing Sheets**



FIG. I



FIG. 2



FIG. 3



FIG. 4



## 1

## ENHANCED GRAVITY CASTING

## FIELD OF THE INVENTION

This invention relates to gravity casting and more specifically to enhanced gravity casting of a molten metal.

## CROSS REFERENCE TO RELATED APPLICATIONS

None

## STATEMENT REGARDING FEDERALLY SPONSORED RESEARCH OR DEVELOPMENT

None

## REFERENCE TO A MICROFICHE APPENDIX

None

## BACKGROUND OF THE INVENTION

The casting of molten metal and particularly molten metals such as molten lead for battery parts is done under different casting conditions. One of the casting methods is high pressure intensification which involves increasing the pressure of molten lead in the cavity by driving a piston into the molten metal to substantially increase the pressure. This process of intensification is described more fully in Ratte U.S. Pat. Nos. 6,202,733; 6,363,996; 6,405,786; 6,499,530; 6,513,570; 6,598,658 and 6,564,853 and uses pressures that compress the metal to reduce the volume of air bubbles in the metal.

Another method of casting battery parts is gravity casting. Gravity casting is preferred for casting larger parts that cool slowly because the gravity casting allows the molten metal to slowly flow under the pressure of gravity to fill any voids in mold cavity as the molten metal solidifies. This results in a part that is substantially free of cracks and voids. Gravity casting uses the head pressure generated by the molten metal to fill out the mold cavity. Thus gravity casting is done at a low fluid pressure within the molten metal. In certain applications, such as larger parts that are immersed in an acid, a gravity cast battery part is highly desirable since the molten metal flows and fills during the solidification process thus virtually eliminating solidification cracks and stresses in the battery part. Since cracks and stresses in a battery part, which is immersed in an acid, can cause rapid deterioration of the battery part it is generally preferred to gravity cast large articles if the article is located in an acid such as found in a battery. However, one of the disadvantages of gravity cast articles is that the articles generally lack the surface definition of high pressure injection molded parts.

The present invention provides an enhanced gravity casting process wherein the molten metal is allowed to solidify under gravity casting conditions while at the same time a follower, which is a portion of the mold surface, is maintained under a following pressure to follow the volume contraction of the molten metal as the molten metal solidifies. That is, as the metal shrinks during solidification the pressure on the molten metal is maintained so that the mold surface or follower moves toward the mold cavity in response to the shrinkage due to solidification. A further feature of the invention is that at the same time air is allowed to escape from the molten metal through a passage which is sufficiently small that molten lead does not flow therest.

## SUMMARY OF THE INVENTION

An apparatus and method for enhanced gravity casting wherein a portion of the mold is maintained in following

## 2

pressure contact with molten metal as it solidifies to allow the mold surface to follow the contraction of the solidifying metal. A further feature of the invention is the use of clearance between mold parts that is sufficient to allow air to escape but insufficient to allow molten metal to flow therest.

## BRIEF DESCRIPTION OF THE DRAWINGS

FIG. 1 is a sectional view of a gravity casting apparatus 10 in a mold filling condition;

FIG. 2 is the sectional view of the gravity casting apparatus of FIG. 1 in a closed condition;

FIG. 3 is an enlarged partial view showing the relationship between a mold inlet passage and a movable mold part; and

FIG. 4 is a partial schematic view of an apparatus for enhanced gravity casting of an article.

## DESCRIPTION OF THE PREFERRED EMBODIMENT

FIG. 1 is a sectional view showing the enhanced gravity casting apparatus 10 comprising a lower mold part 11 and an upper mold part 12 or housing that define a mold cavity 13. That is, mold part 12 includes a fixed mold surface 12a that defines a portion of the top of mold cavity 13 and mold part 11 includes a bottom mold surface 11a that defines the bottom portion of mold cavity 13 and a side mold surface 11b that defines the sides of mold cavity 13. Upper mold part 12 includes a cylindrical inlet passage 14 therein to allow molten metal to flow from a molten metal holding chamber 17 formed in mold part 12. Chamber 17 comprises an open top chamber with a cylindrical sidewall 18 and a converging sidewall or shoulder 19 that connects with an inlet passage 14 to direct molten lead in chamber 17 into the mold cavity 13 under gravity pressure.

Located within chamber 17 is a shutoff member 20 or movable mold part having a cylindrical upper portion 20a, a converging portion or shoulder 20b and a lower cylindrical portion 20c. The diameter of the lower portion 20c is identified by  $D_1$  and the diameter of the inlet passage 14 is designated by  $D_2$ . FIG. 1 shows the movable mold part 20 in the gravity castings condition wherein molten lead 9 is allowed to flow from chamber 17 into the bottom mold cavity 13 under the influence of gravity.

Reference number 24 defines the fluid interface between the molten metal 9 and the air or gas atmosphere above the molten lead. A lead source 25 supplies molten lead to the chamber 17 to maintain a level of molten lead in the chamber 17 so that molten lead can flow into the mold cavity under the gravity pressure on the molten lead. FIG. 1 identifies the pressure  $P_1$  of the molten lead in the mold cavity. The pressure  $P_1$  is due to the head of molten lead above the mold cavity 13.

As can be seen in FIG. 1, the shutoff member 20 is maintained at least partially submerged in the molten lead 9 in chamber 17 and in a spaced condition from the inlet passage 14. It should be understood that the reference to molten lead herein is meant to include lead and lead alloys. As shown in FIG. 1, the molten lead 9 is free to flow into cavity 13 from chamber 17 under the pressure of gravity.

Thus, the first step in the method of enhanced gravity casting includes directing a charge of molten lead 9 into a chamber 17 located in fluid communication with a battery part cavity 13 to generate a gravity pressure on the molten metal, which allows the battery part cavity 13 to fill with molten lead 9 under a gravity flow condition.

This method is particularly useful with large casting and particularly useful with those castings that weight many pounds or have such configurations that the molten lead needs to solidify slowly. As can be seen in FIG. 1, the molten lead 9 is allowed to fill the mold cavity 13 under the gravity pressure on the molten lead.

FIG. 2 illustrates the movable mold part in the solidification or closed condition wherein the mold cavity end surface 20d of shutoff member 20 preferably forms a continuous part of the mold surface with mold surface 12a to define the mold cavity 13 therein. In the solidification condition the moveable mold part 20 remains at least partially immersed in the bath of molten lead 9 with end mold surface 20d of movable mold part 20 forming a closure for the mold cavity 13. In this condition shutoff member 20 is located in the molten lead in chamber 17 and the shutoff member surface 20c is in engagement with a mold inlet passage 14 while the molten lead remains in a liquid state 9. The engagement of the member 20c with the inlet passage 14 prevents further gravity flow of molten lead into the mold cavity 13. In the position shown shoulder 19 functions as a stop for shoulder 20b to prevent further downward movement of member 20. In the preferred position the end face 20d is substantially coextensive with mold face 12a and is prevented from moving into cavity 13 due to the engagement of shoulder 20b and 19.

FIG. 3 is an enlarged partial cross sectional view showing the relationship of the shutoff member 20 and particularly cylindrical surface 20c in relation to the inlet passage 14. In the embodiment shown the movable mold part 20 is maintained in pressure contact with the molten lead 9 through a following force F on the movable mold part 20. The pressure of the metal in the mold cavity is indicated by  $P_2$ . In this condition, the pressure of the metal in the mold  $P_2$  is balancing the following force F on the moveable mold part. As the molten metal solidifies and shrinks the pressure  $P_2$  decreases causing the mold part 20 to be forced downward until the mold pressure again rises to the level  $P_2$  to balance with following force F. Thus, by maintaining a constant following force F on the mold part 20 the mold face 20d can follow the solidification volume contraction of the metal during the solidification process. In the preferred method, upon solidification, the following force F and the time of shutoff are adjusted such that the mold surface 20d is in substantial alignment with mold surface 12a. By following force it is meant that the following force F is sufficient so as to cause the mold surface to move toward the cavity in response to the shrinkage of the metal during solidification but the following force is generally insufficient to compress and deform the metal beyond the internal volume shrinkage that normally occurs during gravity casting. Thus, in the present process the volume of individual air bubbles remaining in the molten metal remain substantially the same since the article is not subject to intensification pressures. However, the present process can also provide for a decrease in the mass of air in the gravity casting by allowing air to escape from the solidifying casting.

Thus, a further feature of the invention is the clearance between the inlet passage 13 of mold part 12 and the movable mold part surface 20c, which is indicated by  $X_0$  in FIG. 3. The clearance  $X_0$  is maintained sufficiently small so that the molten lead does not flow therethrough but sufficiently large so that air in the molten lead can escape therewith. Typically, under gravity casting conditions with molten lead, an air or gas clearance of about 0.005 inches or less is sufficient clearance to allow air bubbles in the molten lead to escape from the solidifying metal but insufficient to

allow molten lead to flow therewith. However, the actual amount of air clearance can vary depending on the shape of the surfaces. In contrast a liquid clearance for a molten metal such as lead or the like to flow therewith is substantially higher under gravity casting conditions.

FIG. 4 shows a view of the present invention wherein the gravity casting apparatus 10 is supplied by molten metal from a source 25 and a two way cylinder 31 having an extendible and retractable arm 33 is shown in engagement with movable mold part 20. Gravity casting apparatus 10 is shown in the down condition or the condition wherein following force F is maintained on member 20 as illustrated in FIG. 2. The dashed lines, which are indicated by 20', show the movable mold part 20 in the retracted or open condition as illustrated in FIG. 1.

Thus in the present invention includes a method of enhanced gravity casting by directing a charge of molten lead into a chamber 17 located in fluid communication with a battery part cavity 13. Next one allows the battery part cavity 13 to fill with molten lead under a gravity flow condition. Once filled one extends a shutoff member 20 located in the molten lead 9 in the chamber 17 into engagement with a mold inlet passage 14 while the molten lead is in a liquid state to close off the inlet passage 14 and prevent further gravity flow of molten lead into the mold cavity 13. By maintaining sufficient following pressure on the shutoff member 20 through member 31 as the molten lead 9 solidifies it allows the shutoff member to follow a solidification volume contraction of the molten lead 9 in the mold cavity 13 to thereby form an enhanced gravity casting where the surfaces features are have high definition and detail.

In the preferred method the end face 20d of shutoff member 20 is brought into substantial alignment with a face 12a of the mold cavity 13 as the volume contraction occurs during the solidification of the molten lead in the battery part cavity by determining the amount of expected volume contraction during the solidification phase.

By forming the shutoff member with a diametrical dimension less than the dimension of the chamber 17, when the shutoff member is in the closed condition, the molten lead can remain in a molten state surrounding the shutoff member 20 and in position where the molten metal can be directed into the mold cavity 13 after the solidified part is removed from the mold cavity 13.

By maintaining the shutoff member 20 and the inlet passage 14 with sufficient air clearance  $X_0$  to permit air to escape from the molten lead in the cavity but insufficient to permit molten lead to escape therewith one can allow air to escape from the molded part and thereby provide a more dense casting without having to compress the air bubbles in the cast part.

In the present process one applies a following force F to the shutoff member through a moveable piston 31 or the like and positions the mold the mold inlet passage 14 on a top side of the battery part cavity 13. In the preferred method the following force F, which is sufficient to cause the mold surface to follow the volume contraction of the solidifying metal, is maintained on the solidifying part when the molten metal is in a liquid state and continues until the solidification process is complete. Thus in the present invention an internal volume reduction due to shrinkage is solely compensated by maintaining a following force on the molten lead until the molten lead solidifies.

A further feature of the invention is that the second mold part is located at least partly in a chamber of molten lead with the chamber 17 in fluid communication with the mold

**5**

cavity 13 and the molten lead 9 in the chamber maintainable in a molten state to permit gravity casting of a second article by removing a first cast part from the mold cavity and replacing the mold part with an empty mold cavity below the chamber.

I claim:

1. A method of enhanced gravity casting comprising:  
directing a charge of molten lead into a chamber located in fluid communication with a battery part cavity;  
allowing the battery part cavity to fill with molten lead under a gravity flow condition;  
forming the shutoff member with a dimension less than the dimensions of the chamber so that when the shutoff member is in the closed condition the molten lead remains in a molten state around the shutoff member  
extending the shutoff member located in the molten lead in the chamber into engagement with a mold inlet passage while the molten lead is in a liquid state to close off the inlet passage and prevent further gravity flow of molten lead into the mold cavity; and  
maintaining a following force to generate sufficient pressure on the shutoff member as the molten lead solidifies to allow the shutoff member to follow a volume contraction of the molten lead in the mold cavity to thereby form an enhanced gravity casting.

2. The method of claim 1 allow and end face of the shutoff member to be brought into substantial alignment with a face of the mold cavity as the volume contraction occurs during the solidification of the molten lead in the battery part cavity.

3. A method of enhanced gravity casting comprising:  
directing a charge of molten lead into a chamber located in fluid communication with a battery part cavity;  
allowing the battery part cavity to fill with molten lead under a gravity flow condition;  
extending the shutoff member located in the molten lead in the chamber into engagement with a mold inlet passage while the molten lead is in a liquid state to close off the inlet passage and prevent further gravity flow of molten lead into the mold cavity;  
maintaining a following force to generate sufficient pressure on the shutoff member as the molten lead solidifies

5

**6**

to allow the shutoff member to follow a volume contraction of the molten lead in the mold cavity to thereby form an enhanced gravity casting; and

maintaining the shutoff member and the inlet passage with sufficient clearance therebetween to permit air to escape from the molten lead in the cavity but insufficient to permit molten lead to escape therewith.

4. The method of claim 1 including the step of applying a following force to the shutoff member through a moveable piston.

5. The method of claim 1 including the step of forming the mold inlet passage on a top side of the battery part cavity.

6. The method of claim 1 including the step of lowering the shutoff member into the fluid inlet passage while molten lead is present in the inlet passage.

7. The method of claim 6 including the step of maintaining a following force on the shutoff member when the shutoff member is in engagement with the inlet passage to permit the shutoff member to follow the volume contraction of the molten lead as the molten lead solidifies.

8. The method of claim 1 wherein an internal volume reduction due to shrinkage is solely compensated by maintaining a following force on the molten lead until the molten lead solidifies.

9. A method of enhanced gravity casting comprising:  
directing a charge of molten lead into a chamber located in fluid communication with a battery part cavity;  
allowing the battery part cavity to fill with molten lead under a gravity flow condition;  
extending a shutoff member to prevent further gravity flow of molten lead into the mold cavity; and  
maintaining a following force to generate sufficient pressure on the molten lead as the molten lead solidifies to cause a follower to reduce a volume of the battery part cavity in direct response to a volume contraction of the molten lead in the mold cavity to thereby form an enhanced battery part gravity casting; and  
maintaining an air clearance but not a liquid clearance between the shutoff member and an inlet passage to the battery cavity.

\* \* \* \* \*